

April 20, 1948.

J. A. M. VAN LIEMPT

2,439,913

METHOD OF TREATING COILED TUNGSTEN FILAMENTS

Filed Feb. 26, 1943.



Inventor:  
Johannes A.M. van Liemt,  
by Vernet C. Gaffman  
His Attorney.

## UNITED STATES PATENT OFFICE

2,439,913

## METHOD OF TREATING COILED TUNGSTEN FILAMENTS

Johannes Antonius Maria van Liempt, Eindhoven, Netherlands, assignor to General Electric Company, a corporation of New York

Application February 26, 1943, Serial No. 477,326  
In the Netherlands October 28, 1941

4 Claims. (Cl. 148—11.5)

1

In the incandescent lamp industry, it has long been the aim to manufacture tungsten wire "glow-bodies" or filaments consisting of large overlapping crystals. This is more important in so-called "spiral" or "coiled-filament" lamps, in which the filament is wound in a helical form, and especially when the filament is helically wound several times (twice or more) into a "coiled-coil," as it is broadly termed. For it has been found that in such lamps the sagging of the filament and the consequent light reduction during the life of the lamp is considerably less when the filament consists of large crystals which generally comprise one or more turns or convolutions of a single coil—or, in the case of a coiled-coil, one or more turns of the first helical coiling—than when the filament shows a fine crystalline structure.

Besides sagging, the amount of vibration-resistance or endurance is of great importance in appraising the quality of a filament. To ascertain the vibration-resistance or life under vibration, one may proceed in the following way. Lamps with filaments whose vibration-endurance is to be determined are burned intermittently while on a vibration-burning-frame, an hour at rated voltage and an hour switched off in alternation. The vibration-burning-frame vibrates, for example, at a frequency of 10 to 50 vibrations per second, and with a very small amplitude, e. g., 0.2 mm. Such vibrations correspond with those to which incandescent lamps are often exposed in normal service, as in the presence of motors and other machinery.

In themselves, filaments with high vibration-endurance are already known. As employed in straight or plain-wire vacuum lamps, for example, they show a very fine structure, because small amounts of thorium oxide have been added to the tungsten. However, such material cannot be used for making coiled or coiled-coil filaments, because it sags badly in service. Carbon filament lamps also show good life under vibration; but these lamps have only low efficiency, and a carbon filament cannot be helically coiled, speaking in a practical sense.

Thus with the materials and methods hitherto used it was not really possible to make a coiled or repeatedly-coiled (coiled-coil) filament that had high vibration-endurance.

The inventor has now discovered that the vibration-endurance of a filament does not depend so much on the size of the crystals of which it is composed, or on the way in which the adjacent crystals are associated or interengaged

2

in the filament, as on the physical character of the internal structure of the individual crystals. He has further found that vibration-resistant filament coils consisting of crystals having an average size of at least one convolution of a single coil or of the first coiling of a coiled-coil can remain quite extensible and can be considerably elongated (at ordinary room temperature of some 20° C.) after recrystallization. By this is to be understood that the length of a single coil can be stretched at least threefold, and the length of a coiled-coil at least sixfold. Ordinary coils consisting of large crystals (which comprise at least one turn of a single coil, or of the first coiling of a coiled-coil) cannot be elongated so much as this after recrystallization; on the contrary, such a thing is only possible before recrystallization takes place. Despite this difference in extensibility, vibration-resistant filaments according to the invention show when etched practically the same structure, under microscopic examination, as the old coiled filaments that do not stand vibration. It is true that the known coiled single-crystal wires are extensible when in an unused lamp; but they lose this property in use. During the coiling, they have undergone a process of deformation, and they will eventually recrystallize while in operation.

As a result of his discovery that the vibration-endurance of a filament depends on the physical character of the internal structure of the individual crystals, the inventor has found that vibration-resistant and very extensible single coil or coiled-coil recrystallized filaments can be made of tungsten wire which naturally gives a recrystallized structure consisting of large crystals, that have at least about an average crystal size of one turn or convolution of a single coil, or of the first coiling in the case of a coiled-coil. It is desirable, furthermore, that the wire material should contain traces of iron, for example, 0.05 to 0.1 per cent by weight, since thus the application of the method or process in accordance with the invention results in greater vibration-endurance of the filaments. The extensible vibration-resistant coiled filaments according to the invention are useful for the electrode or cathode coils of electric discharge devices or tubes, including discharge lamps and especially fluorescent lamps of the ordinary low-pressure positive column type, as well as for the "glow-bodies" of incandescent lamps. Both incandescent lamps and discharge devices are

hereinafter referred to generally and broadly as electric lamps.

The method or process employed may start with coiled filaments without mandrels, which have already undergone the usual "setting" heat treatment for the relief of deformation-stress (in the case of single coils, on iron mandrels, in the case of coiled-coils, on molybdenum mandrels, for example), and from which the mandrels used in the coiling have been removed, as by a chemical method. At this stage, and before being exposed to a temperature of recrystallization or "grain-growth," the filaments are preliminarily subjected to heat treatment between about 1500° C. and 2000° C., with a heating period of at least about 5 minutes. As a result of this, a considerably advanced lattice-restoration or readjustment occurs amongst the filament atoms or molecules, and this readjustment conduces to the desired characteristics of the filaments as regards extensibility and vibration-endurance. To produce this advanced lattice-readjustment, the coils may be heated in a tungsten furnace (for instance) for a period of 5 minutes to two hours, at a temperature of about 1850° C. Naturally, this should be done under protective conditions that insure against any contamination of the tungsten metal, as in an atmosphere of pure, dry hydrogen. The operation can also be carried out in a lamp (in which the filament has been mounted as usual) by aging this lamp (e. g., a 130 volt lamp) for 5 minutes to two hours at an under-voltage (e. g., 70 volts) corresponding to a temperature of 1850° C. Speaking in a general way, the coils should be heated up to the highest possible temperature at which in 5 to 120 minutes recrystallization or grain-growth just does not occur.

After initial treatment at about 1850° C. outside of a lamp, the coils may be fully recrystallized in a tungsten furnace at about 2400° C. (under protective conditions as indicated above), and then mounted in a lamp; or they may be mounted in a lamp first and then burned or aged. For the sake of greater vibration-endurance, the latter method is best, because thus the portions of the filaments in and near the eyelets of the support-wires retain the structure which they acquired during the heating at 1850° C., and do not recrystallize fully; and so such lamps are more resistant under vibration than those whose filaments are completely recrystallized.

When the method of aging in a lamp at an undervoltage is followed, then recrystallization at rated voltage may be effected either directly after this, or when the lamp is put into ordinary use.

Theoretically, the temperature needful for a stated lattice-readjustment and the heating period are interrelated according to the formula:

$$T(13.5 + \log t) = C$$

where  $T$  is the absolute temperature and  $t$  is the time of heating in seconds, while  $C$  as usual denotes a constant. The value of  $C$  depends on the degree of deformation that the metal crystals have undergone, and the kind of tungsten wire. A corresponding curve  $I$  may be drawn with the values of  $\log t$  as abscissas and the values of  $T$  as ordinates. It is obvious that this curve  $I$  crosses the  $T$  axis at a point  $F$  whose ordinate is

$$\frac{C}{13.5}$$

In accordance with this invention, the lattice-readjustment is accomplished in the right-hand

part of the diagram between 1500° C. and 2000° C., with a heating time of 5 minutes to 2 hours; and as the curve  $I$  represents lattice-readjustment, so a certain portion (AE, say) of this curve 5 defines the range that is used according to the invention. This is in contrast with what happens in the case of an ordinary incandescent lamp, where both lattice-readjustment and recrystallization occur (more or less concurrently) at the 10 operating temperature of the lamp or higher: that is, the heating is considerably above the range of mere lattice-readjustment; and in the diagram, it would be above the aforesaid curve  $I$ , generally in the neighborhood of another curve 15  $II$  which expresses the relation between  $T$  and  $\log t$  for recrystallization. Pursuant to the invention, on the other hand, one heats only according to a lattice-readjustment value of  $C$  which is 20 5 per cent to 20 per cent smaller than the recrystallization constant for a heating time of at least 5 minutes, where the recrystallization constant is understood to be equal to the product  $T(13.5 + \log t)$  when the heating time  $t$  in seconds and the temperature  $T$  are so chosen that recrystallization just does take place.

Although the crystal size is affected but little, if at all, by the described method of producing vibration-resistant filaments, very surprisingly 25 the extensibility of the coiled filaments produced according to the invention is much greater than that of filaments manufactured in the usual way. By the method or process according to invention, simple coils can be made which in the recrystallized state can be elongated fivefold, and once-coiled-coils (double-coils) which in that state can be elongated ten to fifteenfold. On the other hand, the extensibility of coils made in the usual way is no more, as a rule, than such that they can be stretched out to double their length. It may 30 be that the greater extensibility of coils according to the invention is a consequence of the fact that they show far fewer crystal faults and spots of irregular current distribution than the coils manufactured in the usual way.

40 Besides the advantage of greater vibration-endurance, very extensible coils present still other advantages. They can, for example, be mounted by machinery with relative ease. They also offer advantages in cases where a filament is stretched 45 out in mounting, as in the manufacture of long tubular incandescent lamps, such as stage or show-window lamps.

What I claim as new and desire to secure by Letters Patent of the United States is:

50 1. A method of treating a coiled tungsten filament wire which when recrystallized consists of crystals of an average size of at least one wire turn, and is thus resistant to sagging, to give the coil high vibration-endurance and high extensibility in the direction of its axis at ordinary room temperature, as contrasted with poor corresponding characteristics without this treatment; which method consists in maintaining the coiled wire at lattice-readjusting temperature until lattice-restoration has been effected before allowing the wire to reach a higher temperature that results in recrystallization.

55 2. A method of treating a coiled tungsten filament wire which when recrystallized consists of crystals of an average size of at least one wire turn, and is thus resistant to sagging, to give the coil high vibration-endurance and high extensibility in the direction of its axis at ordinary room temperature, as contrasted with poor corresponding characteristics without this treatment; which

method consists in subjecting a coiled tungsten wire of this character containing traces of iron of the order of 0.05 to 0.1 per cent by weight to lattice-readjusting heat between 1500° C. and 2000° C. for at least five minutes, and until lattice-restoration has been effected, before subjecting the wire to a higher temperature.

3. A method of forming high vibration-resistant and highly extensible coiled tungsten filament wire, which consists in coiling on a mandrel a tungsten wire which when recrystallized consists of crystals of an average size of at least one wire turn, annealing the mandrel-supported coiled wire to eliminate the deformation strains therein, removing the mandrel from the coiled wire, and then subjecting the coiled wire to a temperature between 1500° C. and 2000° C. for a period of at least five minutes to effect a far advanced lattice-restoration thereof, before subjecting the said coiled wire to a higher temperature at which recrystallization thereof would occur.

4. The method of providing an electric incandescent lamp with a high vibration-resistant coiled tungsten filament, which method consists in coiling a tungsten wire which when recrystallized consists of crystals of an average size of at least one wire turn, annealing the coiled wire to eliminate the deformation strains therein, mounting a

length of the annealed coiled wire in place within the lamp to form the filament thereof, and then operating the lamp at a voltage lower than its rated operating voltage for a period of at least five minutes to subject the filament to a temperature between 1500° C. and 2000° C. and effect a far advanced lattice-restoration thereof before operating the lamp at a voltage at which the filament would be subjected to a higher temperature at which recrystallization would occur.

JOHANNES ANTONIUS MARIA VAN LIEMPT.

#### REFERENCES CITED

The following references are of record in the file of this patent:

#### UNITED STATES PATENTS

| Number    | Name         | Date          |
|-----------|--------------|---------------|
| 1,280,704 | Fuller       | Oct. 8, 1918  |
| 1,815,779 | Karef et al. | July 21, 1931 |
| 1,826,524 | Ramage       | Oct. 6, 1931  |
| 2,114,426 | Laise        | Apr. 19, 1938 |
| 2,165,310 | Spaeth       | July 11, 1939 |

#### FOREIGN PATENTS

| Number  | Country       | Date          |
|---------|---------------|---------------|
| 267,312 | Great Britain | Mar. 17, 1927 |
| 468,449 | Great Britain | July 6, 1937  |